

## 1

2,837,427

### ZINC BASE TERNARY ALLOY CONTAINING TIN AND LEAD

Luigi Monaco, New York, N. Y.

No Drawing. Application May 28, 1956  
Serial No. 587,906

1 Claim. (Cl. 75—178)

This invention is concerned with a novel alloy having 15 specially desirable properties for use in making jewelry of the less expensive kind.

An object of this invention is to provide a novel metal alloy which is easily cast into desired shapes in rubber molds by the usual methods of die casting.

Another object of this invention is to provide a metal alloy which may be cast into articles of jewelry which can be easily plated and soldered.

Still another object of the invention is to provide a metal alloy which is malleable and easily worked.

Still another object of the invention is to provide a

## 2

series of alloys which are easily compounded without special precautions.

The alloy in this invention consists basically of 1. A mixture of zinc, tin and lead.

5 Specifically the formula comprises:

|          | Percent |
|----------|---------|
| (a) Zinc | 70      |
| (b) Tin  | 10      |
| (c) Lead | 20      |

10 This alloy is relatively inexpensive for many uses including the fabrication of jewelry, toys and ornaments and each is simply compounded by melting the ingredients together at the required temperature of 650–700 degrees Fahrenheit. The resulting alloy in each case has to a high degree all of the properties outlined in the objects herein disclosed.

I claim:

An alloy consisting of zinc 70%, tin 10%, lead 20%.

### References Cited in the file of this patent

#### UNITED STATES PATENTS

333,786 Sellon ----- Jan. 5, 1886

#### OTHER REFERENCES

“Revue de Metallurgie” (Dannenmuller) vol 40, pages 85–90 (1943), page 90 relied on.